

# United States Patent Office

2,884,324  
Patented Apr. 28, 1959

1

2,884,324

## MOLYBDENUM-TITANIUM-COBALT ALLOY

George A. Timmons, Ferndale, and Marion Semchyshen, Dearborn, Mich., assignors to American Metal Climax, Inc., a corporation of New York

No Drawing. Application December 6, 1955  
Serial No. 551,228

1 Claim. (Cl. 75—176)

The present invention relates to cast molybdenum-base alloys.

The object of the invention is to provide a molybdenum-base alloy casting capable of being worked at elevated temperatures and having high strength at temperatures in the vicinity of 1600° F.

The alloys of the present invention contain from .10% to .22% titanium, from .05% to .15% cobalt, unavoidable amounts of oxygen not exceeding .005%, small amounts of residual carbon, and the balance molybdenum, except for minute and unavoidable quantities of impurities. The alloys are prepared by arc melting in vacuum, preferably using a furnace of the type disclosed in United States Patent No. 2,656,743. Carbon is added to react with any oxygen present in the raw materials and to leave a slight excess in the final casting. The best results are obtained when the carbon content is less than .04%. The absolute pressure during the melting operation is preferably maintained below 50 microns of mercury.

The raw materials used in making the new alloy consisted of molybdenum powder having an oxygen content

2

ranging from .012% to .029%, titanium sponge having an oxygen content below .2%, cobalt (vacuum melted 99.9% pure cobalt).

Specific examples of the composition of the new alloys include the following:

|    | A               | B       | C       |         |
|----|-----------------|---------|---------|---------|
|    | Percent         | Percent | Percent |         |
| 10 | Titanium.....   | .18     | .15     | .22     |
|    | Cobalt.....     | .11     | .07     | .05     |
|    | Carbon.....     | .03     | .02     | .025    |
|    | Oxygen.....     | .0015   | .001    | .001    |
|    | Molybdenum..... | balance | balance | balance |

Alloy A above was found to have a tensile strength of 94,100 pounds per square inch at 1600° F. in vacuum. This value which is higher than that of any known material indicates that the alloy may be used to advantage where exceptional strength is required at 1600° F. for a short time. The same alloy has a 100 hour creep-rupture strength of 67,000 pounds per square inch at 1600° F., but its strength drops off rapidly on increases in temperature with the result that it is inferior to some other known molybdenum-base alloys in creep-rupture properties at 1800° F. and higher.

25 What is claimed is:

A cast molybdenum-base alloy capable of being worked at elevated temperatures and containing from .10% to .22% titanium, from .05% to .15% cobalt, not more than .005% oxygen, not more than .04% carbon, and the balance consisting essentially of molybdenum.

### References Cited in the file of this patent

### UNITED STATES PATENTS

35 2,678,269 Ham et al. May 11, 1954